

J. F. SANDERS.  
Processes of Amalgamating Ores.

No. 150,793.

Patented May 12, 1874.

Fig. 1.



Fig. 2.



Witnesses.

Chas. Raettig.  
El. Webb

Inventor.

J. F. Sanders  
by his attorney  
A. B. Bresen

# UNITED STATES PATENT OFFICE.

JOHANN F. SANDERS, OF LOUISVILLE, KENTUCKY.

## IMPROVEMENT IN THE PROCESSES OF AMALGAMATING ORES.

Specification forming part of Letters Patent No. 150,793, dated May 12, 1874; application filed April 20, 1874.

*To all whom it may concern:*

Be it known that I, JOHANN FRIEDRICH SANDERS, of Louisville, in the county of Jefferson and State of Kentucky, have invented a new and Improved Process of Treating and Amalgamating Auriferous Ores, of which the following is a specification:

In the accompanying drawing, Figure 1 represents a vertical longitudinal section of the apparatus I prefer to use for carrying my invention into effect. Fig. 2 is a plan or top view of the same.

The apparatus herein illustrated forms the subject-matter of a separate application of a patent, which is filed at the same time with the present.

Similar letters of reference indicate corresponding parts in both figures.

This invention has for its object to reduce as much as practicable the expense of separating gold from the ores or inferior metals containing the same; and consists more particularly in exposing such ores or metals to a blast of hydro-oxygen gas, thereby reducing or oxidizing the ores, vaporizing the gold, and thus by vaporization bringing the gold into condition for condensation and convenient separation, the vapors being carried over a sheet of water, which lies on a bed of quicksilver, so that the water will condense the vapors and carry the products of condensation in contact with the quicksilver, which will properly amalgamate the gold. The invention also consists in a new chemical means of treating the molten ore in the furnace, for separating in the furnace the molten gold from the molten quartz or silicium which will not vaporize, all as hereinafter more fully described.

By practical experiments I have ascertained that a blast of hydro-oxygen gas will give the greatest amount of heat for the purpose of reducing or oxidizing the ores, and that such blast has the greatest chemical effect, next to the light of the sun, on said ores. A blast of the kind named can be used at will either as a reducing-blast by melting the ore and absorbing in the form of vapor the metallic constituents of the ore from the non-vaporizing quartz

or silicium and other non-vaporizing constituents; or, it can be used as an oxidizing-blast for oxidizing all the baser metals and separating therefrom in the form of vapor the gold that was mixed with such baser metals. In the first case—that is to say, for a reducing-blast, it is necessary to use about two volumes of hydrogen gas to one volume of oxygen gas; while in the second case—that is to say, for an oxidizing-blast, a surplus of oxygen gas is necessary, or oxygen gas alone may be used. These gases are obtained by suitable processes well known in the arts and sciences, and I do not consider it necessary to give the formula for making the same.

The gases are, through a proper tuyere, A, conducted into the interior of the furnace B, which interior contains the ore to be reduced. The gases on being ignited melt the contents of the furnace and carry away with them through the passage A the vaporized products of combustion, in which invariably the larger proportion of the gold contained in the ores will be carried off. These vapors are conducted through a passage, a, into a trough or vessel, C, which contains at its bottom a bed, D, of quicksilver, upon which a sheet, E, of water is placed. Cold water is, through a pipe, b, continuously sprinkled or conducted into this vessel C, the surplus water escaping through openings d at one end. The cold-water spray coming from above, as indicated, passes through the vapors that are escaping from the furnace, and serves to force such vapors more or less into contact with the cold water, to cool and condense the same and separate from them the condensed particles of gold which fall upon the surface of the water in the form of fine spray. For further insuring the proper absorption of the gold contained in the vapors, a transverse plate, e, is formed in the vessel C, whereby the vapors are carried very close to the surface of the water. Finally, the vapors that have been deprived of all the gold contained in them are carried off through a pipe or chimney, f. The gold that enters the water E passes through the same by its gravity into contact with the quicksilver D, and is absorbed by the quick-

silver, owing to the chemical affinity of this metal for gold, while the other metals that may have been condensed from the vapor, and all other solid substances that may have reached the quicksilver, will remain between the quicksilver and water without combining with the quicksilver. It is then only necessary to draw off the quicksilver after the process has been continued for a certain length of time, and to separate from it, by the well-known processes now usually followed, the gold that was absorbed by it. In order to prevent all the non-auriferous products of condensation which pass through the water and do not fall through the quicksilver from forming a film between the quicksilver and water, and preventing the gold from reaching the quicksilver, a proper stirring apparatus may be employed within the vessel C, so that the contact of the water with the quicksilver may never be entirely interrupted. Gases that escape through the pipe or chimney f may, if they are supposed to contain valuable ingredients, such as sulphur, &c., be conducted into suitable apparatus for further utilization. The furnace B should be properly heated by the blast before the ore is put into it, an opening, h, being formed in the top of the furnace for admitting theores, said opening being subsequently closed by a proper plug. It must be observed that the quartz or silicium that is contained in the ore cannot be changed into vapor by this blast, but it fuses readily under the influence of the blast, and by fusing sometimes carries small particles of gold along with it; and in order to separate this gold from the fused quartz or silicium I add about two to six parts of oxide of lead (litharge) or galena (sulphate of lead) to one part of the gold which is supposed to be in the charge. This oxide or sulphate of lead, when molten, becomes lead, which has in the molten state the same degree of affinity for molten gold which quicksilver in the cold state has for cold gold. I employ the oxide or sulphate of lead, and not pure lead, because the melting-degree of the latter is too low. The gold will, when thus treated, be absorbed by the lead, and it will by the lead also be carried to the bottom of the furnace. When it is supposed that a proper quantity of such lead charged with gold is contained at the bottom of the furnace, the silicium or quartz is poured off, a new charge put into the furnace, and the smelting-process continued as before. The process of sublimation and concentration is then renewed until the furnace

is nearly filled with concentrated metals—that is to say, with the lead containing the gold. A surplusage of oxygen gas is then used in the blast, for oxidizing the lead and all other base metals that may be in the mass contained within the furnace, and the precious metal will then be vaporized and separated from the lead, and carried away into the vessel C, there to be condensed, in the same manner already described. This process of oxidation goes on very rapidly, and care must be taken that the temperature in the furnace is not too high during oxidation. In fact it should not be higher than to bring the mass to a quiet boiling-point, and to prevent it from spattering spontaneously. When the lead is all oxidized it hardens, and becomes a litharge-powder, and a molten mass of nearly pure gold, having a brilliant metal shine and a slightly greenish color, remains in the furnace, and can be poured off or vaporized, as before. The reducing process, at first described, is now resumed. Admixtures of all other metals that may be contained in the ores enter partly in combination with the silicium when the same is in a liquid state, and are, when the oxidizing-blast is admitted into it, oxidized, and do not, therefore, enter into amalgamation with the quicksilver. Therefore, the gold will be very rapidly and cheaply separated from all the metals and other minerals contained in the ores, and the desired effect obtained. I may state that in carrying this process into effect a series of furnaces, of substantially the construction shown, may be used, and the residuum in one furnace may be partly or entirely resubmitted to action in another furnace, and so on, until the entire separation of the gold shall have been effected—as far, at least, as such separation is at all practicable.

I claim as my invention—

1. The process of separating gold from the ores by vaporizing it, and conducting the vapors over a sheet of water that rests on a bed of quicksilver, substantially as and for the purpose described.
2. The process herein described of separating, by the oxidizing-blast, the gold from the oxide of lead which was used to separate it from the molten quartz or silicium, as described, and of subsequently recovering the gold from the vapors by condensation, in the manner described.

Witnesses: J. F. SANDERS.  
A. V. BRIESEN,  
E. C. WEBB.